

## UNITED STATES PATENT OFFICE

1,986,001

## MANUFACTURE OF PLASTERS

Victor Lefebure, Hampstead, London, England

No Drawing. Application September 5, 1930,  
Serial No. 479,931. In Great Britain October  
10, 1929

## 8 Claims. (Cl. 106—34)

In my U. S. A. Patent Specification No. 1,879,877 it is shown how natural anhydrite, formerly a waste material of no value for plaster making, can be converted into a good plaster. I have now found other ways of making new forms of anhydrite plasters which have distinct commercial advantages.

According to this invention I provide a process of manufacture of anhydrite plasters which consists in mixing anhydrite with the hemihydrated form of calcium sulphate,  $\text{CaSO}_4 \frac{1}{2} \text{H}_2\text{O}$ , which is the standard chemical composition of plaster of Paris.

If a standard plaster, such as plaster of Paris or one of the well-known forms of so-called "hard plasters", containing  $\text{CaSO}_4 \frac{1}{2} \text{H}_2\text{O}$  be diluted with fillers such as powdered silica or gypsum the mass after setting becomes correspondingly weak and soft according to the amount of dilution, which result would be expected in the dilution of cements and binders with inert fillers in general. But if ground anhydrite be employed instead of fillers such as the above it does not act as a diluent but for a given concentration gives a much harder and stronger mass.

The following example illustrates the invention, the parts being by volume.

Example.—One part of plaster of Paris is mixed with eight parts powdered silica; the resulting mass after setting with water in the usual way, is very weak and soft, quite unusable as a plaster. One part of the same plaster of Paris and eight parts ground anhydrite, after treating in the same manner with water, give a mass as hard and strong as the neat plaster of Paris.

Another important advantage of the process of manufacture according to this invention is the increase in speed of setting, and improvement in properties of standard wall plasters by the addition of anhydrite, or of "accelerated" anhydrite. By the latter I refer to such anhydrite plasters as are covered by the patent mentioned above, or any similar accelerated anhydrites. If, for example, a standard wall plaster with a set of about one hour be mixed with anhydrite which has practically no setting properties, or with an "accelerated" anhydrite plaster setting in about one hour, the resultant product when set in the usual way, and, within certain

proportions of mixture, will set in from less than one minute up to fifteen minutes, much quicker than either of the components. For example, a mixture of one part of medium setting hard wall plaster with a set of about one hour, mixed with two parts of anhydrite plaster arranged to set in about one hour will set to a hard mass almost instantaneously, in from less than one minute to two or three minutes, varying with conditions such as temperature and excess water.

Although this observed effect of increased speed has been found true in general in the admixtures of anhydrite or accelerated anhydrite with hemihydrated plasters there will be some forms of the latter in which the increase of speed, although substantial may not be so great. For example, in admixtures of accelerated anhydrite with Keene's cement, which is not wholly a hemihydrated plaster in view of its double and higher temperature roasting, the speed may be reduced from four hours down to about 25 minutes, but not necessarily down to one minute.

Thus the method can be employed to increase the setting speed of slow wall plasters, or, by heavy loading with anhydrite, to reduce the speed of quick moulding plasters, thus producing plasters of equal or better quality than standard plasters at substantially lower cost, the material added being simply ground mineral anhydrite, or the latter with a trace of low-priced catalyst.

As an example, the standard hemihydrated calcium sulphate has a very quick set. In this form it is used for moulding as plaster of Paris. In the industry organic retarders are used to reduce the speed. According to this invention, it is possible to reduce the speed, making this plaster suitable for wall purposes by adding high percentages of anhydrite, such as, for example, one part of plaster of Paris to eight parts of anhydrite. I have found that the quickest mixtures, which are almost instantaneous, consist of one volume of the hemihydrated form with from about one half to three volumes of accelerated anhydrite. At some points between these proportions, varying with the raw materials, there is a peak of speed.

The following table gives the variation of speed with admixture employing a standard commercial retarded hemihydrated plaster and an accel-

5

10

15

20

25

30

35

40

45

50

erated anhydrite, both setting individually in about 60 minutes:—

| Percent standard plaster | Percent accelerated anhydrite | Setting time |
|--------------------------|-------------------------------|--------------|
| Nil.                     | 100                           | Minutes      |
| 10                       | 90                            | 60           |
| 20                       | 80                            | 15           |
| 40                       | 60                            | 4            |
| 50                       | 50                            | 2½           |
| 60                       | 40                            | 1            |
| 80                       | 20                            | 2½           |
| 100                      | 0                             | 60           |

and the following table gives the variation employing the same standard plaster and non-accelerated anhydrite with a practically indefinite setting time:—

| Percent standard plaster | Percent non-accelerated anhydrite | Setting time      |
|--------------------------|-----------------------------------|-------------------|
| Nil.                     | 100                               | No practical set. |
| 10                       | 90                                | 15 minutes.       |
| 20                       | 80                                | 6 minutes.        |
| 40                       | 60                                | 6 minutes.        |
| 80                       | 20                                | 24 minutes.       |
| 100                      | Nil.                              | 60 minutes.       |

The slowest mixtures are obtained by heavy dilution with the unaccelerated anhydrite. This gives a very satisfactory and easily standardized method of controlling speed of set without the addition of undesirable organic substances, or without loading with high percentages of inorganic accelerators.

These mixtures have various other advantages besides those mentioned above: First, the set mass from the mixture when using the accelerated anhydrite, is as hard and strong as (in fact, almost invariably harder and stronger than) the normal hemihydrated plaster in the mixture when used alone. In using high percentages of non-accelerated anhydrite the resultant set mass is not always harder and stronger, but makes as good practical plaster up to very high dilution. Secondly, the anhydrite content of the mixture improves the final product in the direction of the properties of anhydrite plasters, not only as regards hardness and strength, but as regards a surface more suitable for rapid after decoration. Thirdly, the normal method of producing very rapid anhydrite plasters is to increase the setting or accelerating agent percentage, which increases cost. The mixtures according to the present invention, enable very fast plasters up to a practically instantaneous set, to be made at lower cost, employing in the combination either anhydrite alone or anhydrite with very small percentages of setting agent. Another advantage which has been observed is that for practical use mixtures can be obtained which have a higher sand-carrying capacity than the two components, certainly as regards the initial strength of the mass as distinguished from the ultimate strength, which is a point of considerable practical importance.

The manner in which the invention is applicable to various requirements is further illustrated by the following examples, which are by no means limitative of the field of usefulness of the invention.

#### Example 1.—Wall plaster

A plaster suitable for wall surfaces in normal building operations made by the mixture of one part of standard retarded hemihydrated plaster, having a firm set of about 60 minutes, with 9 parts of anhydrite containing 0.2% of potassium sulphate and zinc sulphate salts in molecular proportions, having itself a firm set of about 5 hours. This resultant mixed wall plaster has a firm set of about 60 minutes, being of average speed for wall work.

#### Example 2.—Casting or moulding plaster

A plaster suitable for very quick work, made by mixing one part by volume of a standard retarded hemihydrated plaster with 4 parts by volume of anhydrite containing 2% of potassium sulphate and zinc sulphate mixed salts in molecular proportions.

What I claim and desire to secure by Letters Patent is:—

1. A plaster composition consisting of two components only in which the first component consists of unburnt natural anhydrite ( $\text{CaSO}_4$ ), and the second component consists of burnt gypsum ( $\text{CaSO}_4 \cdot \frac{1}{2}\text{H}_2\text{O}$ ), in the proportions of 1-9 parts of the first component to 1 part of the second.

2. A plaster composition consisting of two components only in which the first component consists of accelerated unburnt natural anhydrite ( $\text{CaSO}_4$ ), and the second component consists of burnt gypsum ( $\text{CaSO}_4 \cdot \frac{1}{2}\text{H}_2\text{O}$ ).

3. A plaster composition consisting of two components only in which the first component consists of unburnt natural anhydrite ( $\text{CaSO}_4$ ), and the second component consists of a retarded  $\text{CaSO}_4 \cdot \frac{1}{2}\text{H}_2\text{O}$  wall plaster.

4. A plaster composition consisting of two components only in which the first component consists of accelerated unburnt natural anhydrite ( $\text{CaSO}_4$ ), and the second component consists of a retarded  $\text{CaSO}_4 \cdot \frac{1}{2}\text{H}_2\text{O}$  wall plaster.

5. A plaster composition consisting of two components only in which the first component consists of accelerated unburnt natural anhydrite ( $\text{CaSO}_4$ ), and the second component consists of a retarded  $\text{CaSO}_4 \cdot \frac{1}{2}\text{H}_2\text{O}$  wall plaster.

6. A plaster composition consisting of two components only having a firm set of about 1 hour, in which the first component consists of unburnt natural anhydrite containing about 0.2% of potassium sulphate and zinc sulphate in molecular proportions, having a firm set of about 5 hours, and the second component consists of a retarded  $\text{CaSO}_4 \cdot \frac{1}{2}\text{H}_2\text{O}$  wall plaster having a firm set of about 1 hour.

7. A plaster composition consisting of two components only having a rapid set of 1-5 minutes in which the first component consists of unburnt natural anhydrite containing about 2% of potassium sulphate and zinc sulphate in molecular proportions, and the second component consists of a retarded  $\text{CaSO}_4 \cdot \frac{1}{2}\text{H}_2\text{O}$  wall plaster.

8. A plaster composition consisting of two components only in which the first component consists of unburnt natural anhydrite ( $\text{CaSO}_4$ ), and the second component consists of a wall plaster of the Keene's cement type, i. e. an accelerated dead-burnt gypsum plaster.

VICTOR LEFEBURE.